

## UNITED STATES PATENT OFFICE.

WILLOUGHBY STATHAM SMITH, OF BENCHAMS, HENRY JOSEPH GARNETT, OF LYMNE, AND JOHN ANCEL HOLDEN, OF SUNNYSIDE, ENGLAND.

## REFINEMENT OF NICKEL ALLOYS.

No Drawing. Application filed May 3, 1928, Serial No. 274,959, and in Great Britain April 25, 1927.

This invention relates to the refinement of nickel alloys consisting mainly of nickel, that is, alloys which contain 50% or more of nickel, and the balance may be any one or 5 more of the following elements:—iron, chromium, tungsten, vanadium, molybdenum, silicon, aluminium, copper, cobalt, titanium or zirconium.

The object of this invention is to minimize 10 or substantially eliminate the sulphur content.

It is well known that nickel alloys are very difficult to work when they contain even a 15 small percentage of sulphur; amounts of as little as .03% in certain alloys are very injurious.

If pure virgin metals are melted into alloys 20 in furnaces in which there is no contamination and the alloys are subsequently worked by ordinary commercial processes, contamination by sulphur is almost inevitable. Such operations as preheating for rolling or for 25 forging in gas or coal fired furnaces lead to an absorption of sulphur, which is necessarily confined to the surface of the material. When 30 the rolled or forged scrap is returned to the furnace for melting, a small increment of sulphur is made to the charge. During the course of time this increment becomes greater, 35 till eventually the material contains so much impurity that it cannot be worked as perfectly as the pure alloy.

According to this invention the furnace 40 charge consisting for example, of virgin metal with scrap or entirely of scrap is melted in 35 the presence of a slag and hydrogen or other reducing atmosphere. A suitable slag consists mainly of lime with silica, and a small amount of either fluorspar or calcium chlo- 45 ride may be used. Preferably the furnace is of the induction type, using low, medium or high frequency.

It has been found that fifteen minutes refining with a slag of the composition mentioned, in an atmosphere as described, will 45 reduce the sulphur content very considerably in an alloy containing 80% of nickel. The hydrogen supply is then cut off and the slag removed from the surface of the metal, and 50 before a new slag is formed, a small amount of an oxide of one of the constituents of the alloy or other metals is introduced. For example, in the case of a nickel iron alloy, an oxide of iron— $Fe_2O_3$  or  $Fe_3O_4$ —may be in-

troduced. In the case of nickel-iron-copper 55 alloys, a small addition of copper oxide may be used, and so on. As this addition is in amounts of less than 1% and the quantity of oxide reduced is only a fraction of 1%, its effect upon the chemical composition of the 60 alloy can be ignored.

The added oxide is allowed to re-act for a few minutes and then a new slag is formed from suitable materials, such as broken glass, etc. The molten metal is then ready for pour- 65 ing.

It is possible however after removal of the hydrogen directly to tem the metal from the crucible but if so it will be found that during freezing a large volume of hydrogen is 70 evolved and in consequence the resulting ingots are honeycombed. Even with the use of de-gasifying agents, such as manganese, magnesium, silicon and the like, the resulting bars are worthless. They can, how- 75 ever, be remelted in the ordinary way and made into sound workable ingots (because the hydrogen is expelled during freezing), but this is not so economical as the method de- 80 scribed above.

Additions of a suitable finishing agent such as magnesium are made in the usual manner.

What we claim is:—

1. A method for the refinement by mini- 85 mizing the sulphur content of nickel alloys having a nickel content of 50% or more, which consists in melting the furnace charge in the presence of a slag and an atmosphere of hydrogen, and subsequently after removal of the reducing atmosphere adding an oxide of 90 one of the constituent metals to absorb the absorbed hydrogen.

2. A method for the refinement by mini- 95 mizing the sulphur content of nickel alloys having a nickel content of 50% or more, which consists in melting the furnace charge in the presence of a slag and hydrogen, cut- 100 ting off the supply of hydrogen after about fifteen minutes and then adding a small amount of an oxide of one of the constituents of the alloy for removing the absorbed hydro- gen.

In testimony that we claim the foregoing as our invention we have signed our names this 18th day of April, 1928.

WILLOUGHBY STATHAM SMITH.  
HENRY JOSEPH GARNETT.  
JOHN ANCEL HOLDEN.